

## UNITED STATES PATENT OFFICE

2,145,020

## NICKEL-CHROMIUM ALLOYS

Frederick M. Becket, New York, and Russell Franks, Niagara Falls, N. Y., assignors to Electro Metallurgical Company, a corporation of West Virginia

No Drawing. Application June 15, 1938,  
Serial No. 213,816

2 Claims. (Cl. 75—171)

This invention concerns nickel-chromium alloys. Such alloys have been used for a long time and have served well in resisting corrosion and deterioration at high temperatures. They are suitable for heating elements because of their high electrical resistivity and their excellent resistance to oxidation. As a rule, the alloys contain at least 60% nickel and 10% or more chromium. In some instances, iron has been present in a percentage as high as 15%, while in others it has been held to a much lower percentage.

The forging of ingots of such alloys is often difficult. By careful control of the melting practice, and by the use of appropriate deoxidizers, the forgeability of the alloy ingots can be improved to a considerable degree, but even under the most carefully controlled conditions some difficulty is encountered from tearing, checking, and cracking of the ingot during the hot working operations. To obtain a product of high quality it is necessary to grind the partially forged ingot frequently to remove such defects.

We have found that improved hot working properties can be imparted to the nickel-chromium alloys by the addition of columbium in relatively small proportions, for example about 0.40%. Some improvement occurs when the columbium content is as low as 0.20%, and it is unnecessary to add more than 2% columbium. We do not definitely know why columbium improves the hot working properties of the alloys, although it has been observed that the alloy ingots treated with columbium do not pipe to as great an extent as those that contain no columbium, even though the alloys have been otherwise melted and deoxidized in the same manner. The columbium addition produces a definite refinement in grain size, which undoubtedly influences the hot working properties of the metal. As shown in the accompanying Table No. I, the alloys treated with columbium possess a higher degree of ductility and toughness in the hot-rolled condition, which means that, inherently, the alloys treated with columbium would have less tendency to tear or check when deformed either hot or cold.

TABLE I

| Metal No. | Composition (remainder Fe) |            |            |            |           |            | Izod impact, ft.-lb. | 5  |
|-----------|----------------------------|------------|------------|------------|-----------|------------|----------------------|----|
|           | Percent Cr                 | Percent Ni | Percent Mn | Percent Si | Percent C | Percent Cb |                      |    |
| 1         | 12.9                       | 77.4       | 2.05       | 0.20       | 0.06      | None       | 74                   |    |
| 2         | 12.7                       | 77.9       | 2.11       | 0.22       | 0.06      | 0.43       | 113                  |    |
| 3         | 12.6                       | 74.8       | 2.01       | 0.32       | 0.05      | 1.11       | 83                   | 10 |
| 4         | 12.2                       | 74.4       | 1.95       | 0.29       | 0.06      | 2.02       |                      |    |
| 5         | 20.5                       | 77.5       | 0.44       | 0.63       | 0.06      | None       | 70                   |    |
| 6         | 20.9                       | 74.6       | 1.52       | 0.34       | 0.09      | 0.59       | 78                   |    |

Tensile tests on metal, as hot rolled, thousands of pounds per square inch

|   | Yield point | Tensile strength | Percent elongation in 2 inches | Percent reduction in area | 20 |
|---|-------------|------------------|--------------------------------|---------------------------|----|
| 1 | 58.0        | 76.5             | 9                              | 31                        |    |
| 2 | 66.0        | 106.7            | 34                             | 57                        |    |
| 3 | 52.0        | 106.0            | 38                             | 63                        |    |
| 4 | 64.0        | 111.5            | 35                             | 54                        |    |
| 5 | 57.0        | 96.0             | 16                             | 23                        |    |
| 6 | 56.0        | 103.0            | 20                             | 26                        | 25 |

These improvements are obtained without a sacrifice of resistance to corrosion or oxidation at elevated temperatures. Tests have shown that alloys treated with columbium have approximately the same low rate of oxidation, when heated in air at 1050° to 1150° C., to alloys made under the same conditions but containing no columbium. This is demonstrated by data of Table II.

TABLE II

| Metal No. | Composition (rest Fe) |            |            |            |           |            | Percent loss in weight of sample held 72 hrs. at 1150° C. in air | 40 |
|-----------|-----------------------|------------|------------|------------|-----------|------------|------------------------------------------------------------------|----|
|           | Percent Cr            | Percent Ni | Percent Mn | Percent Si | Percent C | Percent Cb |                                                                  |    |
| 7         | 13                    | 74.2       | 1.85       | 0.07       | 0.05      | None       | 1.51                                                             |    |
| 2         | 12.7                  | 77.9       | 2.11       | 0.22       | 0.06      | 0.43       | 1.65                                                             |    |
| 3         | 12.6                  | 74.8       | 2.01       | 0.32       | 0.05      | 1.11       | 2.19                                                             |    |
| 4         | 12.2                  | 74.4       | 1.95       | 0.29       | 0.06      | 2.02       | 1.73                                                             | 45 |

Accordingly, the invention comprises a nickel-chromium alloy containing 10% to 30% chromium, 0.2% to 2% columbium, iron in an amount not exceeding 15%, the remainder nickel which

50

may include incidental impurities and residual deoxidizers. Preferably, the chromium content is between 15% and 25% and the iron content is less than 5%.

- 5 The nickel-chromium alloys of the invention may be deoxidized, before the addition of the columbium, with manganese or silicon, or with other deoxidizers such as calcium, aluminum, zirconium, or titanium. Residual deoxidizer other than silicon and manganese should not exceed about 1%; manganese is preferably less than 3% and the silicon is preferably less than 1%. The low percentages of phosphorus and sulphur and other incidental impurities usually

present in commercial alloys of this type may also be present in the metal of the invention.

We claim:

1. Alloy having substantially the composition: 10% to 30% chromium, 0.2% to 2% columbium, iron in an amount not exceeding 15%, the remainder nickel. 5

2. Alloy resistant to oxidation and deterioration at high temperatures and composed substantially of 15% to 30% chromium, 0.2% to 2% columbium, iron in an amount less than 5%, the remainder nickel. 10

FREDERICK M. BECKET.  
RUSSELL FRANKS.